

## UNITED STATES PATENT OFFICE

2,676,917

## METHOD OF MAKING CORROSION RESISTANT ARTICLES HAVING A BRIGHT SURFACE

Milton B. Hammond and Glade B. Bowman,  
Edgeworth, Pa., assignors, by mesne assignments, to Rockwell Spring and Axle Company, Coraopolis, Pa., a corporation of Pennsylvania

No Drawing. Application May 15, 1952,  
Serial No. 288,048

3 Claims. (Cl. 204--36)

1

This invention relates to a method of making corrosion resistant articles having a bright surface.

Until recently, corrosion resistant articles having bright surfaces, as for example automobile bumpers and automobile body trimmings, have been made by electrodepositing a layer of nickel or copper and nickel on a steel base, and then electrodepositing a thin layer of chromium such as ten millionths of an inch of chromium on the nickel layer. The nickel layer was of a thickness between a minimum of about .0015" and a maximum of about .0035", averaging about .0025". Such articles had a bright surface and would withstand corrosion in the standard salt spray test for about 96 hours.

Recently due to the critical shortage of nickel, a government regulation has issued requiring that the thickness of the nickel layer average not over .001". An article having a nickel layer .001" thick and a layer of chromium ten millionths of an inch thick on top of the nickel layer, will withstand corrosion in the standard salt spray test for only about 24 to 48 hours, and accordingly, for many purposes is unsatisfactory.

Schoonmaker and Stockton Patent 2,315,740 owned by the assignee of this application, discloses a method of making corrosion resistant articles which do not have bright surfaces. According to one embodiment of the patent, a layer of nickel is electrodeposited on a steel base, then a layer of zinc is electrodeposited on the nickel, and thereafter the article is heat treated to a temperature sufficient to cause the nickel to alloy with the zinc. In carrying out the heat treating, the article is usually heated at a temperature of about 700° F., although this temperature may vary between about 300° F. and a temperature substantially above the melting point of zinc. The patent points out that nickel and zinc form alloys having different proportions of nickel and zinc, that the gamma and gamma prime alloys contain in the neighborhood of 80% zinc and 20% nickel, that the gamma and gamma prime alloys have high corrosion resisting characteristics, and that the best practice in carrying out the nickel-zinc alloying heat treatment is to employ temperatures and times which develop the gamma and gamma prime nickel zinc alloys.

While articles made according to the Schoonmaker and Stockton patent have good resistance to corrosion when subjected to the standard salt spray test, they have a dull surface rather than the bright surface which is required for certain

2

uses. If an article is made according to the patent, and a layer of chromium is applied to it without first buffering the article, the product does not have a bright surface. The chromium deposit disappears when subjected to salt spray for about 12 hours. If the product of the patent is first given a light buffering in order to remove any excess zinc which may be present and to produce a bright surface, and then chromium is electrodeposited on the bright surface, the surface of the chromium plated article will be bright, but the article still will only resist the corrosion of the salt spray for about 12 hours.

We have discovered a method whereby bright surfaces which will withstand the standard salt spray test for a period of time of the order of 100 hours can be produced while limiting the average thickness of the nickel layer to less than .001".

In carrying out our invention, we electrodeposit a layer of nickel on any metal or alloy base on which nickel can be electrodeposited. A preferred base material is steel. The nickel layer should have a thickness of at least .00005", it being unimportant, except from a cost standpoint, as to what the upper limit of the thickness is. Usually, however, the thickness of the nickel layer is between .00005" and .0015", a preferred thickness for the nickel layer being .0004". A layer of zinc is then electrodeposited on the nickel layer, the zinc layer being at least .000005". There is no upper limit to the thickness of the zinc layer except as a matter of economy. Usually the thickness of the zinc layer is between .00001" and .0005", a preferred thickness of the zinc layer being .0001".

The electrodeposit is then buffed for a time sufficient to cause all of the zinc to penetrate into and alloy with the nickel, and to give a bright surface. The buffering may be carried out by the use of an ordinary cloth buffering wheel using an ordinary buffering compound such as a lime buffering compound. The pressure employed in buffering may be the same as is commonly used for the buffering of nickel. As an example, buffering has been accomplished satisfactorily employing a cloth buffering wheel having a diameter of about 14" and a width of about 5", by employing a total pressure of 135#, the wheel rotating at a speed of about 1750 R. P. M.

The extent of buffering required in order to cause all of the zinc to penetrate into and alloy with the nickel and to give a bright surface, can be readily determined by the color of the electrodeposit. The article which has been plated with nickel and then with zinc has a white or milky

color due to the zinc deposit. During buffing, this white color gradually disappears so that when all of the zinc has alloyed with the nickel and there is no free zinc on the surface, the article has the slightly brown cast or appearance of the nickel. After the article has been buffed to the extent indicated, it is electroplated with chromium, as for example a chromium plate having a thickness of ten millionths of an inch. An article made in the manner described, employing a nickel layer having a thickness of .0004" and a zinc layer having a thickness of .0001", buffed as described, and then plated with ten millionths of an inch of chromium, has been found to withstand the corrosion of the standard salt spray test for a period of time of the order of 100 hours. In contrast to this result, an article plated with .0004" of nickel and then plated with ten millionths of an inch of chromium, without using any zinc layer, will withstand the standard salt spray test only for about 12 hours.

The buffing employed according to our invention removes some of the zinc layer and causes the rest of it to penetrate into and become alloyed with the nickel layer. The pressure used and the heat developed during the buffing are such that the nickel flows during the buffing operation.

It is believed that the improved results accomplished according to the present invention, as compared with chromium plating an article obtained according to the Schoonmaker and Stockton patent wherein the nickel and zinc are caused to alloy by heating without any buffing action, are due to the fact that buffing produces a different nickel-zinc alloy from that produced by mere heating. For instance, a steel plate was electroplated with a layer of nickel .0004" thick, then with a layer of zinc .0001" thick, and then buffed in the manner described until all of the zinc had penetrated into and alloyed with the nickel layer. The surface of the buffed article was analyzed and was found to contain about 12% zinc and about 88% nickel. It is believed that the good adherence of the chromium deposit made according to our method in which buffing is employed to cause the zinc to penetrate into and alloy with the nickel, is due to the presence of a nickel-zinc alloy containing a relatively small proportion of zinc and a relatively large proportion of nickel and having a slightly brown cast or appearance, as contrasted with the gamma nickel-zinc alloy containing about 80% of zinc and 20% of nickel and having a blue cast or appearance, produced by heating in accordance with the Schoonmaker and Stockton patent. In any event, greatly improved results are obtained by following our method since, when a product is made according to the patent and chromium plated and subjected to salt spray, the chromium disappears when subjected to the standard salt spray test for a period of about 12 hours.

In carrying out our method, the preferred base to which the nickel is applied is steel, but the base may be aluminum, copper, brass, bronze, zinc, or any ferrous or non-ferrous metal or alloy on which nickel can be plated.

We prefer that the article which has been plated with nickel and then with zinc, not be heated before buffing. We have carried out a series of tests in which steel plates were coated with nickel and then with zinc. One of these plates was not heated before buffing. Others were heated for seven minutes at temperatures of 350° F., 500° F. and 700° F. We found that the plate which was not heated required the least buffing,

and that as the heating temperature before buffing was increased, more buffing was required in order to produce a surface which, after plating with chromium, satisfactorily resisted salt spray corrosion.

So far as the thickness of the zinc layer is concerned, while a thickness of .0001" is preferred, satisfactory resistance to corrosion has been obtained with a zinc layer as thin as .000005". No harm is done by employing a zinc layer greatly exceeding .0001" thick, since it simply means that the buffing will have to be continued for a longer time in order to remove excess zinc and to cause the remaining zinc to penetrate into and alloy with the nickel, which of course is uneconomical.

The chromium plating can be done by the use of a standard chromium plating bath operated under standard conditions. It can be a chromium sulphate bath containing 45 ounces per gallon of CrO<sub>3</sub> and 0.45 ounce per gallon of SO<sub>4</sub>. The plating may be carried out at a temperature of about 118° F. employing a cathode current density of about 100 amperes per square foot. The thickness of the chromium layer is not critical. Since all chromium plating is somewhat porous, it is not relied upon to impart corrosion resistance to the article but is used simply to provide a bright surface.

The invention is not limited to the preferred embodiment, but may be otherwise embodied or practiced within the scope of the following claims.

We claim:

1. The method of making a corrosion resistant article having a bright surface, which comprises electrodepositing on a metal base a layer of nickel having a thickness of at least .00005", electrodepositing on the nickel layer a layer of zinc having a thickness of at least .000005", buffing the deposit for a time sufficient to cause all of the zinc to penetrate into and alloy with the nickel and produce a bright surface, and electrodepositing a layer of chromium on the bright surface.

2. The method of making a corrosion resistant article having a bright surface, which comprises electrodepositing on a steel base a layer of nickel having a thickness of .00005"-.0015", electrodepositing on the nickel layer a layer of zinc having a thickness of .00001"-.0005", buffing the deposit for a time sufficient to cause all of the zinc to penetrate into and alloy with the nickel and produce a bright surface, and electrodepositing a layer of chromium on the bright surface.

3. The method of making a corrosion resistant article having a bright surface, which comprises electrodepositing on a steel base a layer of nickel having a thickness of about .0004", electrodepositing on the nickel layer a layer of zinc having a thickness of about .0001", buffing the deposit for a time sufficient to cause all of the zinc to penetrate into and alloy with the nickel and produce a bright surface, and electrodepositing a layer of chromium on the bright surface.

#### References Cited in the file of this patent

#### UNITED STATES PATENTS

| Number    | Name               | Date         |
|-----------|--------------------|--------------|
| 2,315,740 | Schoonmaker et al. | Apr. 6, 1943 |

#### FOREIGN PATENTS

| Number  | Country       | Date          |
|---------|---------------|---------------|
| 474,559 | Great Britain | Nov. 3, 1937  |
| 593,763 | Great Britain | Oct. 24, 1947 |